

A. C. Rand,  
Covering Whips,  
No 78,129. Patented May 19, 1868.

Fig. 1



Fig. 2.



Witnesses.  
A. B. Smith  
J. P. Buckland

Inventor  
A. C. Rand

# United States Patent Office.

A. C. RAND, OF WESTFIELD, MASSACHUSETTS.

Letters Patent No. 78,129, dated May 19, 1868.

## IMPROVED PROCESS OF COVERING WHIPS.

The Schedule referred to in these Letters Patent and making part of the same.

TO ALL WHOM IT MAY CONCERN:

Be it known that I, A. C. RAND, of Westfield, in the county of Hampden, and Commonwealth of Massachusetts, have invented a new and improved Process of Covering Whips; and I do hereby declare that the following is a full, clear, and exact description thereof, reference being had to the accompanying drawings, making a part of this specification, and to the letters of reference marked thereon.

In the manufacture of whips, one or more coverings of thread are wound or braided upon the whip-stock, which latter is generally formed of whalebone and strips of wood, glued together and shaped to form a tapering and springing body for the whip.

The first or inner covering is also, sometimes, formed of narrow strips of cloth, which is afterwards covered by a braided layer of thread.

Various methods have been attempted for protecting the compound stock from moisture, so as to prevent the glue from softening and the parts of the stock from becoming separated, such as painting the stock before any covering is applied, using strips of water-proof or rubber cloth for winding the stock, and applying a water-proof solution directly to the stock or braided covering, which latter method is described in Letters Patent, No. 65,917, granted to Gamaliel King, June 18, 1867.

My process consists in applying, to a whip-stock, thread which has been saturated with a suitable water-proofing solution, and which is wound or otherwise applied to the stock before such solution is dry upon the thread, the winding, in the practical application of the process which I describe herein, being performed immediately after the immersion of the thread in the solution, and upon the same machine.

My process is equally applicable to the winding of a second or outer covering upon the whip, as to the inner covering.

In applying my invention, I have used an ordinary whip-winding machine, with an attachment for containing the water-proofing solution and properly saturating and operating upon the thread.

A machine suitable for such purpose is shown in the aforesaid drawings, in which—

Figure 1 is a plan view of said machine, and

Figure 2 is a side elevation, showing the side at which the operator is stationed when winding.

Said machine consists of the bed A, legs A' A', and the winding-apparatus thereon.

The shaft E turns in bearings in the standards C' C', and has a fast pulley, D; and loose pulley, D', upon it, and a head, F, in which is a socket, for receiving the large end of the whip-stock which is to be wound.

Spring-pins are arranged in this head, to enter the socket and hold the stock, so that it will revolve with the shaft.

In the bar H, which is supported on the standards G G, is formed a tapering groove, which is semicircular in section, and of a length equal to or greater than the length of the stock a, and of depth sufficient to receive about one-half the thickness of a, as shown in fig. 1.

In the ordinary process of winding whips, in a machine of the general construction described, the whip-stock a is inserted and secured in the head F, and the latter is made to revolve by power applied to the fast pulley D.

The operator, after attaching the end of the thread to the stock at the point where the winding is to commence, allows the thread to be drawn between his thumb and finger, and guides it in regular courses upon the stock, sliding the hand along the bar H at the same rate as the winding of the stock proceeds.

To expedite the process, several threads are run out, side by side, at the same time.

For applying my process, I attach to the machine the two rods, m m', which serve as ways, upon which the holder b slides, the latter being attached to the ways by the metallic straps n n, which are looped to grasp the rods m m'.

The holder I construct of sheet metal, of a length greater than its width, and of any convenient form.

The roller e is arranged in the holder, and also the clamp e e, which holds the wiper f.

The wiper consists of two pieces of sheet rubber, or any material which will remove the drip from the saturated thread which passes up through the wiper at *i*.

To move the holder and thread along the ways, as the winding progresses, the handle *h* is attached to the holder.

If a sufficient quantity of some water-proofing mixture be poured into the holder *b*, the machine can be used for applying my process.

I have employed, for saturating the thread, a composition formed of the following ingredients, in the proportions named, to wit:

Caoutchouc, two and a quarter pounds.

Benzine, one gallon.

Linseed-oil, three quarts.

Venice turpentine, half a pint.

White zinc, thirty pounds.

I do not confine myself to the solution named, as any preparation which will impart to the thread the requisite pliability and adhesiveness, while being wound, and will cause it to form, when wound, a close covering, smooth, and impervious to moisture, or nearly so, when dry, can be employed.

Various preparations for the same purpose may be compounded and applied, as before set forth, with satisfactory results.

Having put a sufficient quantity of the water-proofing mixture into the holder to cover the roller *c*, I draw the thread or threads which are to be wound upon the stock, from a bobbin near at hand, and pass it or them beneath the roller and through the wiper, and thence draw it to the stock and attach it thereto.

The stock is then made to revolve, and the holder moved along by means of the handle *h*, until the whole or a sufficient length of the stock has been wound.

The holder is to be replenished from time to time, so as to keep the surface of the mixture above the roller *c*.

In the application of my process, I do not confine myself to the mechanical devices shown, or the composition of the water-proofing mixture as described, but I believe that the application, to a whip-stock, or to the covering already wound thereon, of thread previously saturated with a water-proofing solution, and wound upon the stock, or a covering thereof, while freshly saturated therewith, is a new and valuable improvement in the process of covering whips, and also possesses many advantages over the processes of forming a water-proof covering upon whips by painting, or applying a coating directly to the stocks, or the thread upon them, inasmuch as all waste of the water-proofing material is prevented, and much labor is also avoided, it being difficult to apply the composition smoothly and evenly with a brush or by immersing the stock in it.

It is also much neater in practical use, saturates the thread more thoroughly, and completes in a better manner and at one operation the work which would otherwise require two or more operations, if the water-proofing mixture is applied by brushing or immersion.

The whips wound by my process are also deemed to be superior in poise and quality to whips manufactured by the ordinary processes.

Having described my invention, what I claim as new therein, and desire to secure by Letters Patent, is—

The process of covering whips, substantially as herein specified.

In testimony whereof, I have hereunto set my hand, this twenty-eighth day of December, A. D. 1867.

A. C. RAND.

Witnesses:

J. P. BUCKLAND,

N. B. SMITH.